

## UNITED STATES PATENT OFFICE

2,076,595

## PREPARATION OF VISCOSE SYRUPS

George A. Richter, Berlin, N. H., assignor to  
 Brown Company, Berlin, N. H., a corpora-  
 tion of Maine

No Drawing. Application August 26, 1933,  
 Serial No. 687,016

## 1 Claim. (Cl. 260—100)

This invention relates primarily to the preparation of viscose syrups or cellulose xanthate solutions for the manufacture of artificial silk and sheet material, the sizing of paper and textile fabrics and various other technical uses.

In my application Serial No. 679,585, filed July 18, 1933, I have described the advantages of subdividing or reducing cellulose to a fine or pulverulent condition and then causing it to react directly in the presence of both caustic soda solution and carbon bisulphide to yield a viscose syrup of the desired strength of composition. In that application, I have further pointed out that the caustic soda solution requisite for the desired objective may be of much lower than mercerizing strength, that is, the 18% caustic soda solution customarily employed for the production of a completely xanthatable soda-cellulose. The present invention is centered about a modification of the general practice disclosed and claimed in that application and is aimed to facilitate the subdivision of the cellulose while at the same time leading to a preferred form of subdivided cellulose for the xanthating reaction without, however, requiring additional steps or reagents.

In accordance with the present invention, subdivision or reduction of the cellulose to a fine or pulverulent condition is performed in a wet way, that is, in the presence of water. More specifically, the sub-division of the cellulose is accomplished in the presence of water containing part or all of the caustic soda designed to enter into the subsequent xanthating reaction. Such practice is advantageous in that it makes possible a reduction of cellulose pulp to the desired degree of fineness with good efficiency and with little, if any, hydration or gelatinization of the pulp fibers. Indeed, by using the caustic soda necessary for the subsequent xanthating reaction as a solution of the appropriate strength and/or at the appropriate temperature, hydrating or gelatinizing action on the pulp fibers can be substantially prevented.

It is possible to produce a satisfactory viscose solution by my inventive procedure generally as follows. A suitable cellulose pulp may be subdivided in the presence of a caustic soda solution in a ball or roller mill, a beater or Jordan, or other equivalent impact and/or cutting machine. When the ultimate objective is a viscose syrup containing about 7% caustic soda and 7% cellulose, the proportions of caustic soda, cellulose and water appropriate for such syrup may be added and mixed as raw materials. If desired, however, the

caustic soda and cellulose may be put through the sub-dividing step at higher concentrations; and, after the desired sub-division of the cellulose has been effected, a dilution of the mass with water may be effected. For instance, I may charge the sub-dividing machine with a 10% suspension of fiber in a 10% caustic soda solution and, after the desired sub-division of cellulose has been effected, the suspension may be diluted with water to a causticity of about 7% and carbon bisulphide added thereto to effect xanthation. In another instance, I may initially form a 7% suspension of starting cellulose in a caustic soda solution of mercerizing concentration, say, 18% or greater concentration, whereupon after the desired subdivision of the cellulose has been effected in such solution, a portion of the mercerizing liquor may be separated from the sub-divided cellulose and water added to the suspension to reach the desired composition, say, caustic soda and cellulose contents of 7% each. This latter practice may be advantageous in the case of cotton or linen rags or long-fibered cellulose pulps which require extensive or prolonged sub-division before the desired fineness of cellulose particle is reached, as a mercerizing liquor inhibits the generation of hydrated or gelatinized cellulose even when such extensive sub-division must be accomplished.

While effecting sub-division of the cellulose, the suspension may be artificially refrigerated so as to minimize hydration or gelatinization of the cellulose especially when the caustic soda solution is one which does not mercerize at ordinary or room temperatures. Ordinarily, the lowering of temperature in an aqueous suspension of cellulose fiber being beaten tends to promote a hydrating or gelatinizing action on the cellulose. In consequence of the presence of alkali during the subdivision of the fibers, however, this tendency is reversed, that is, the alkali present in the refrigerated water tends to more than offset the otherwise prevalent hydrating or gelatinizing action. The carbon bisulphide necessary to effect xanthation may be added while sub-division of the cellulose is going on so as to react upon and dissolve finely divided or powdered cellulose as it is progressively being generated in the ball mill, beater engine, jordan, or other impact or cutting machine. As a rule, however, particularly when viscose solutions of about 6% to 8% cellulose content are in view, it is preferable to add the carbon bisulphide after the desired fineness of cellulose has been attained so as to avoid difficulties. Otherwise, the desired mixing action is impeded and the reduction of the unreduced cellulose fibers re-

tarded, since the resulting viscous cellulose xanthate acts more or less like a lubricant and protecting material for the unreduced cellulose fibers. Accordingly, the carbon bisulphide is, as already indicated, preferably added at a late stage or at the conclusion of the cellulose-sub-dividing operation. When high cellulose content is desired in the finished viscose syrup, I start with a cellulose pulp of low solution viscosity as explained in my already-mentioned patent application. It may be well to again observe that the caustic soda solution, in which subdivision of the cellulose pulp is effected, may be cooled to temperature conditions conducive to more or less mercerization. For instance, the pulp may be subdivided in a caustic soda solution of, say 6% to 7% concentration at temperatures in the vicinity of, say, 0° C. In such instance, some mercerization takes place at the low temperature, but when the solution is brought to the preferred xanthating temperature, as should be done, it no longer possesses mercerizing activity. In this connection, it should further be noted that the steps of my process may be carried out at different temperatures. Thus, as already indicated, the sub-division of the fibers may advantageously be performed at low temperatures, e. g., temperatures approaching 0° C. to minimize hydrating or gelatinizing action and/or to promote mercerization in a solution which is non-mercerizing at ordinary or room temperatures. Thereupon, however, the suspension sub-divided cellulose may be permitted to rise in temperature to that of the surrounding atmosphere, say, 20° to 30° C., so as to permit of xanthation to best advantage, that is, without producing undesirably thick or coagulated viscose syrups. Indeed, xanthation may take place with the suspension of fine cellulose at higher temperatures, for instance, at temperatures appreciably above 30° C., in which case a "ripened" viscose syrup can be realized. When viscose is ripened, there is a progressive splitting off of water and sulphur to render the cellulose xanthate less stable, that is, more precipitable by acidic reagents, strong salt solutions, or by mere standing when the temperature of the heat-ripened syrup is not reduced quickly and drastically. Accordingly, when the viscose syrup is produced hot or is heat-ripened, it should be quickly and drastically cooled to effect further reactions such as would give rise to spoilage on account of gelling or coagulation.

The principles of my invention are not limited to sub-division of cellulose without hydration or gelatinization, but sub-divided cellulose in a substantially unhydrated state has been found to undergo smoother and quicker xanthation and is hence preferred. It is, however, a concomitant desirable result of sub-dividing cellulose more particularly in the presence of comparatively strong and/or cold caustic soda solution that hydration is minimized and that the reduction of the fiber to a fine state proceeds most efficiently. It might be observed that the cellulose pulp used as raw material may be partially subdivided while dry and then admixed with the caustic soda solution and sub-divided to the fineness requisite for xanthation. Such a two-stage sub-dividing operation may be preferable when the starting fibrous material is of such long fiber length that dry-grinding is more effective at the beginning than wet-grinding. For instance, such long fibers as manila and cotton when ground in a mill as by rods or balls tend to "spin" or tangle into knots or clumps, whereas, when ini-

tially sub-divided to a proper degree while dry, they can then be more easily and uniformly reduced to the ultimate fineness desired in a wet way, that is, in the presence of caustic soda solution. In some instances, the fiber may be initially cut or ground in the presence of alkali-free water and the last stage of grinding or cutting performed in the presence of a caustic soda solution which represses hydration to an undesirable degree such as ensues, for example, in the production of glassine papers and such as detracts from the smoothness and rapidity of the xanthating reaction. If desired, the fiber used as raw material may have undergone previous mercerization, in which case the fiber has substantially no hydrating tendencies when it is subjected to subdivision in water.

A typical example of procedure accordant with my invention may be practiced as follows. A low viscosity cellulose fiber may be used as raw material, for instance, refined wood pulp or cotton which has undergone treatment with permanganate solution or other solution-viscosity-lowering reagents as disclosed in my already-mentioned application. A fiber thus treated may yield, when dissolved in a cuprammonium solution, a viscosity approximating that of a cuprammonium solution similarly prepared from cellulose which has been converted into soda cellulose and allowed to age in accordance with standard viscose-making practice. The low viscosity fiber may be mixed with caustic soda and water in such proportions as to yield a 7% cellulose suspension in an 8% caustic soda solution. The suspension may be charged into a ball or roller mill of proper construction wherein metal or other suitable balls or rollers serve as the grinding or impact elements. The charged mill may then be caused to rotate slowly and thus to grind or powder the pulp fibers progressively by the pounding action of the balls or rollers. When the fibers have been reduced to particles of a size passing through a fine mesh sieve, say, one of about 200 mesh, carbon bisulphide may be added to the suspension in the proportion of three parts by weight to five parts of the cellulose, on a dry basis. The addition of the carbon bisulphide may be made while the cellulose suspension is in the impact or cutting machine or after the suspension has been delivered to a reaction vessel wherein the xanthating reaction is to take place. In any event, adequate mixing is effected to bring the carbon bisulphide into contact with substantially all of the cellulose particles. Xanthation is allowed to continue and the temperature of the reacting mass is permitted to rise gradually to, say, 27° C. The period for complete xanthation is usually about three hours at the end of which time an amber-colored syrup of surprising clarity is had. Such a syrup has the appropriate cellulose and caustic soda concentration for spinning into artificial silk or casting into pellicles of regenerated cellulose. Should it be desired to change the ratio of alkali and cellulose in the syrup when it is to serve for other than spinning or casting purposes, this may be done by adding water or concentrated caustic soda to the syrup. When the syrup is intended for spinning purposes, it should first be ripened or matured. This may be done in the usual way by keeping the viscose at, say, 20° C., for three to four days; or it may be accelerated by heat treatment such as I have already described. It will, of course, be understood that the time required for sub-dividing the

cellulose preliminary to xanthation may vary, depending upon the size of the charge and the design of the cellulose-sub-dividing machine. Thus, the sub-division of cellulose to a particle size of finer than about 200 mesh may take from about two to four hours in the usual commercial ball mill. It will be understood that the cellulose need not necessarily be ground or pulverized to such fineness of particle size as 200 mesh, although such fineness is preferable from the standpoint of ensuring a smooth, quick and substantially complete xanthation into viscose syrups of the best clarity.

It is possible to use cellulosic material or pulps of a wide variety of characteristics in the practice of my invention. For instance, one may start with chemical wood pulps, such as sulphite or kraft pulp, or wood pulps which have been refined to high alpha cellulose content, e. g., an alpha cellulose content of at least about 93%. In the preparation of viscose syrups of light color intended for such purposes as the manufacture of artificial silk or sheets of regenerated cellulose, it is preferable that the cellulose pulp employed as raw material be white and of high alpha cellulose content so as to conduce to ultimates of the best appearance and physical qualities. Cellulose pulps of other than wood origin, such as cotton, manila, ramie, cotton and linen rags, etc., may also be employed as raw material. In the case of waste rags, reclaimed waste papers, and other impure forms of cellulose, the initial reducing step of my process in the presence of caustic soda solution may be accompanied by a considerable consumption of caustic soda in reacting upon and dissolving non-alpha cellulose components associated with the cellulose. In such case, the consumed caustic soda may be replaced by other caustic soda at the completion of the sub-dividing operation so as to ensure a causticity in the wet, sub-divided cellulose permissive of a substantially complete xanthating reaction to produce a viscose syrup of the desired composition. In such case, too, the caustic soda solution, particularly if practically exhausted of free alkali, may be partially or completely separated as by washing from the sub-divided cellulose whereupon the sub-divided cellulose may be commingled with a caustic soda solution to produce a properly xanthatable mixture. Such latter practice is preferably adopted when considerable impurities are dissolved in the caustic soda solution present during the sub-division of the cellulose and when it is desired to attain viscose syrups of the best qualities.

The sub-division of the cellulose in the presence of caustic soda is preferably performed in a machine whose material of construction is not affected or reacted upon by the alkali to produce undesirable contamination of the finished viscose syrup. To this end, the material of construction of the cellulose-sub-dividing machine may be chrome-steel alloy, nickel or chromium-plated steel or other metals or alloys resistant to the action of caustic soda and sulphur-containing compounds. The same holds true with the reaction vat in which the sub-divided cellulose may be xanthated after delivery from the sub-dividing machine. My invention although of particular utility in connection with the preparation of viscose syrups may be applied to other cellulose derivatives in connection with which soda-cellulose must be produced. Thus, the preparation of various cellulose ethers like ethyl and methyl cellulose ethers involve the preparation of soda-cellu-

lose as part and parcel of the etherifying process. In such case, the soda-cellulose mixture or combination may be produced accordant with my invention in much the same way as the mixture is prepared for a xanthating reaction. Owing to the lack of a generic expression for the various derivatives into which soda-cellulose may enter, in accordance with my invention, I shall adopt for convenience of designation the expression "soda-cellulose derivative" as the generic expression in the appended claim.

The principles of the present invention may be extended to the preparation of cellulose derivatives or esters like cellulose nitrate and cellulose acetate which, rather than calling for the use of alkali-cellulose during the esterifying operation, require that the cellulose be substantially free from alkali. In such case, the cellulose pulp employed as raw material may be advantageously reduced to fine particle size in the presence of distinctly alkaline water, for instance, a caustic soda solution, thereby repressing the hydration of the pulp fibers during such reduction. The resulting suspension of fine cellulose particles may be washed substantially free of alkali and be substantially completely dried before undergoing conversion into esters like cellulose nitrate or cellulose acetate or into other cellulose derivatives. I am aware of the fact that in my Patent No. 1,842,689, dated January 26, 1932, I have disclosed the advantage of mercerizing cellulose pulp to destroy its hydratability before the pulp fibers are subjected to a pulverizing operation in the presence of water, but when the reducing or pulverizing operation is performed as herein disclosed in the presence of distinctly alkaline water, it is possible to work to advantage with unmercerized cellulose pulp and in the presence of non-mercerizing alkaline solutions. In other words, when alkali is associated with the pulp fibers while they are being mechanically reduced or powdered, it is possible to repress hydration of the pulp fibers by the presence of an alkaline solution of comparatively low alkalinity and without refrigerating the solution, whereas the destruction of the hydratability of cellulose pulp by mercerization before the pulp is subjected to a pulverizing operation in the presence of water necessarily involves the more expensive expedient of using caustic soda solution of sufficiently high strength or one artificially refrigerated to a sufficiently low temperature to exercise a mercerizing action.

I have already indicated that the cellulose xanthate solution may be formed at higher than the desired concentration and then diluted with water, or that it may be increased in causticity. When, however, the suspension of fine cellulose particles in the caustic soda solution is such as to be incompatible with the realization of a cellulose xanthate solution of about 6% to 7% cellulose and about 6% to 10% caustic soda concentration, such as might be desired for spinning or casting purposes, I may add to the suspension not only carbon bisulphide to effect xanthation but such additional water, caustic soda, and fine cellulose particles as may be necessary to produce a cellulose xanthate solution of the desired cellulose and caustic soda concentration. When the suspension of fine cellulose particles has been produced in a caustic soda solution of a strength greater than that desired in the xanthating reaction, for instance, a solution of about 18% or greater strength, such solution may be removed from the suspension and replaced by water so as to lower the caustic soda concentration to the de-

sired value of about 6% to 10%, whereupon carbon bisulphide may be mixed with the diluted suspension to form the solution of cellulose xanthate.

I claim:

- 5 A process which comprises mechanically subdividing cellulose to a particle size of about 200 mesh in water containing sufficient caustic soda dissolved therein and under conditions substantially to prevent hydration or gelatinization of the

cellulose, proportioning the cellulose, water, and caustic soda in the conduct of the process to yield an aqueous suspension of cellulose particles of caustic soda and cellulose contents of about 7% each, and mixing carbon bisulphide with the resulting suspension to form a solution of cellulose xanthate.

GEORGE A. RICHTER.